

Sept. 22, 1931.

H. AEBLY

1,824,524

PROCESS OF PRODUCING IMPREGNATED IRREGULAR PAVING

Filed Jan. 5, 1929

*Fig. 1*



*Fig. 2*



Inventor

Hans Aebly  
by *Donald D. Peeling*  
Attorney

## UNITED STATES PATENT OFFICE

HANS AEBLY, OF ZURICH, SWITZERLAND

## PROCESS OF PRODUCING IMPREGNATED IRREGULAR PAVING

Application filed January 5, 1929, Serial No. 330,676, and in Switzerland January 10, 1928.

The attempt has been made recently to create a road covering by the combination of the road paving with broken stones, abandoned at present, with the modern cold impregnating with asphalt, this new road covering fulfilling the conditions of the modern road traffic. In the literature a process of producing a road of broken stones has been described consisting in that large irregular broken stones are placed in coarse aggregate. The rough road is then rolled, covered with aggregate, poured over with cold asphalt and rolled solid after repeated strewing with aggregate.

15 A great inconvenience of this process consists in the circumstance, that the coarse aggregate serving as foundation for the broken stones, is much too permeable for the cold asphalt owing to the relatively wide intervals between the several small stones. The cold asphalt sinks, in the aggregate, very rapidly down, for the greatest part to the foundation, where it is lost as useless. The rapid sinking down causes further an irregular distribution of the cold asphalt, which will not be substantially improved even by subsequent rolling, as the latter is incapable to still further move the individual stones of the aggregate. These properties of the 20 coarse aggregate are the reason that the cold asphalt does not arrive or only unsufficiently on the lower sides of the broken stones and on the downwardly inclined sides of the same. The embedding of the broken stones remains 25 therefore imperfect, this being of prejudicial influence upon the durability of the cover.

This invention has for its object, to obviate the inconveniences of the process mentioned 30 by using, instead of the coarse aggregate, sand or a fine material of similar behaviour as support for the irregular paving stones. Cold asphalt soaks only very slowly into moistened and compressed sand, as can be 35 easily proved; it penetrates into the sand really only at the subsequent rolling owing to the shaking and pressing of the paving stones. The cold asphalt flows therefore at the utmost to the depth up to which the shaking and pressing acts, i. e. to the just de-

sirable depth, a further flowing down would mean a loss of this expensive material. The mixture of sand and cold asphalt forms a viscid paste, which at the pressing carried out in the usual manner is forced up into the intervals between the paving stones and sucked down again. The cold asphalt plays then the part of a sliding medium for the sand particles. It has been found, that the cold asphalt arrives really also on the lower side of the paving stones. These paving stones are therefore enveloped in the desired measure by the sand-asphalt-mortar which hardens subsequently.

55 An embodiment of the invention is illustrated in the accompanying drawings in which:

Fig. 1 shows the improved road pavement in top plan view.

Fig. 2 is a cross-section of Fig. 1.

The old road or the finished foundation *a* is covered with a layer *b* of sand about 6 cins. thick. In this sand the irregular paving stones *c* are inserted so that the largest, and plainest side is on the top.

70 In this manner an irregular joint system is formed (Fig. 1). Then follows wet rolling for equalizing smaller unevenesses and which at the same time makes the sand rise up to a certain height between the stones. Without waiting for the drying abundant cold asphalt is poured on. Before the setting of the fine dispersing asphalt solution the paving is covered with aggregate, and rolled again. The rolling serves, on the one hand for obtaining a good mixing of the cold asphalt with the sand serving as support and, on the other hand, to effect a complete embedding of the paving stones in the mortar which is thus produced. The strewn on aggregate is 75 designed to prevent smearing of the road roller and to secure a complete filling of joints. After the complete setting of the cold asphalt the sand-asphalt-mixture forms a hard, compact filling *d* of the joints, solidly 80 cementing the paving stones and very resistant against wear. The filtering in of water is thereby prevented and also the formation of holes leading to bursting. Of the kinds of cold asphalt those are specially suited which 85

contain the bituminous substances in colloidal distribution. The advantages of the new process are as follows:—

- 1.—Utilization of the cheaper sand instead of an embedding foundation for the paving stones of aggregate.
- 2.—Avoiding of losses of cold asphalt from too deep soaking.
- 3.—More perfect embedding of the paving stones.
4. A greater impermeability to water, as the paste-like sand-asphalt-mortar completely fills the joints.

I claim:—

- 15 A method of paving street or road surfaces, which consists in depositing upon the bed of the surface a base layer of sand, laying upon the sand paving stones of irregular form and thereby producing a haphazard arrangement of spaces or joints between the stones, subjecting the stones to rolling pressure to level the stones at the top and to depress the stones in the sand and cause the sand to rise in the spaces or joints to a level between the top and bottom surface of the stones, floating over the surface cold liquid asphalt in quantity to fill the joints to the surface level therewith and to form with the sand a viscous pasty mixture, spreading aggregate over the surface before the asphalt sets, and rolling the surface to force the surface asphalt and aggregate down into the joints and to force the pasty mixture of asphalt and sand upward between the stones so as to fill 35 all voids and to form with the aggregate a hard compact filling solidly cementing the stones together.

In testimony whereof I affix my signature.  
HANS AEBLY.

40

45

50

55

60

65